



US006197220B1

(12) **United States Patent**  
Blok et al.

(10) **Patent No.:** US 6,197,220 B1  
(45) **Date of Patent:** Mar. 6, 2001

(54) **CONDUCTIVE POLYMER COMPOSITIONS  
CONTAINING FIBRILLATED FIBERS AND  
DEVICES**

(75) Inventors: **Edward J Blok**, Wadsworth; **Prasad Khadkikar**, Seville; **Jeffrey A. West**, Bellville; **Mark R. Scoular**, Medina; **Joseph V. Rumler**, Strongsville, all of OH (US)

(73) Assignee: **Therm-O-Disc Corporation**, Mansfield, OH (US)

(\*) Notice: Subject to any disclaimer, the term of this patent is extended or adjusted under 35 U.S.C. 154(b) by 0 days.

(21) Appl. No.: **09/588,337**

(22) Filed: **Jun. 6, 2000**

(51) Int. Cl.<sup>7</sup> ..... **H01B 1/24; H01C 7/02**

(52) U.S. Cl. ..... **252/511; 252/512; 252/513;  
252/514; 338/22 SD**

(58) Field of Search ..... **252/512, 513,  
252/514, 511; 264/614, 616, 617; 338/21,  
22 R, 22 SD**

(56)

**References Cited**

**U.S. PATENT DOCUMENTS**

|           |         |                     |         |
|-----------|---------|---------------------|---------|
| 4,833,305 | 5/1989  | Mashimo et al. .... | 219/549 |
| 5,250,226 | 10/1993 | Oswal et al. ....   | 252/500 |
| 5,382,384 | 1/1995  | Baigrie et al. .... | 252/511 |
| 5,643,502 | 7/1997  | Nahass et al. ....  | 252/511 |
| 5,651,922 | 7/1997  | Nahass et al. ....  | 252/511 |
| 5,837,164 | 11/1998 | Zhao ....           | 252/500 |
| 5,985,182 | 11/1999 | Zhao ....           | 252/511 |

Primary Examiner—Mark Kopec

(74) Attorney, Agent, or Firm—Harnes, Dickey & Pierce, P.L.C.

(57)

**ABSTRACT**

The invention provides polymeric PTC compositions and electrical PTC devices with higher voltage capability and improved electrical stability. Depending on device design, the composition can be used in low to high voltage applications 6 volts up to 240 volts.

**38 Claims, 1 Drawing Sheet**





FIG. 1.



FIG. 2.

## CONDUCTIVE POLYMER COMPOSITIONS CONTAINING FIBRILLATED FIBERS AND DEVICES

### BACKGROUND OF THE INVENTION

The invention relates generally to polymeric positive temperature coefficient (PTC) compositions and electrical PTC devices. In the invention relates to polymeric PTC compositions containing fibrillated fibers which exhibit improved over voltage capabilities and an enhanced PTC effect.

Electrical devices comprising conductive polymeric compositions that exhibit a PTC effect are well known in electronic industries and have many applications, including their use as constant temperature heaters, thermal sensors, low power circuit protectors and over current regulators for appliances and live voltage applications, by way of non-limiting example. A typical conductive polymeric PTC composition comprises a matrix of a crystalline or semi-crystalline thermoplastic resin (e.g., polyethylene) or an amorphous thermoset resin (e.g., epoxy resin) containing a dispersion of a conductive filler, such as carbon black, graphite chopped fibers, nickel particles or silver flakes. Some compositions additionally contain flame retardants, stabilizers, antioxidants, antiozonants, accelerators, pigments, foaming agents, crosslinking agents, dispersing agents and inert fillers.

At a low temperature (e.g. room temperature), the polymeric PTC composition has a contiguous structure that provides a conducting path for an electrical current, presenting low resistivity. However, when a PTC device comprising the composition is heated or an over current causes the device to self-heat to a transition temperature, a less ordered polymer structure resulting from a large thermal expansion presents a high resistivity. In electrical PTC devices, for example, this high resistivity limits the load current, leading to circuit shut off. In the context of this invention  $T_s$  is used to denote the "switching" temperature at which the "PTC effect" (a rapid increase in resistivity) takes place. The sharpness of the resistivity change as plotted on a resistance versus temperature curve is denoted as "squareness", i.e., the more vertical the curve at the  $T_s$ , the smaller is the temperature range over which the resistivity changes from the low to the maximum values. When the device is cooled to the low temperature value, the resistivity will theoretically return to its previous value. However, in practice, the low-temperature resistivity of the polymeric PTC composition may progressively increase as the number of low-high-low temperature cycles increases, an electrical instability effect known as "ratcheting". Crosslinking of a conductive polymer by chemicals or irradiation, or the addition of inert fillers or organic additives may be employed to improve electrical stability.

In the preparation of the conductive PTC polymeric compositions, the processing temperature often exceeds the melting point of the polymer by 20° C. or more, with the result that the polymers may undergo some decomposition or oxidation during the forming process. In addition, some devices exhibit thermal instability at high temperatures and/or high voltages that may result in aging of the polymer. Thus, inert fillers and/or antioxidants, etc. may be employed to provide thermal stability.

Among the known inert fillers employed in PTC polymeric compositions are polymeric powders such as polytetrafluoroethylene (e.g., Teflon™ powder), polyethylene and other plastic powders, fumed silica, calcium carbonate,

magnesium carbonate, aluminum hydroxide, kaolin, talc, chopped glass or continuous glass, fiberglass and fibers such as Kelvar™ polyaramide fiber (available from DuPont) among others. According to U.S. Pat. No. 4,833,305 by 5 Machino et al., the fibers employed preferably have an aspect ratio of approximately 100 to 3500, a diameter of at least approximately 0.05 microns and a length of at least approximately 20 microns.

Polymeric PTC materials have found a variety of 10 applications, such as self-regulating heaters and self-resettable sensors to protect equipment from damage caused by over-temperature or over-current surge. For circuit protection, the polymeric PTC devices are normally required to have the ability to self-reset, to have a low resistivity at 15 25° C. (10 Ωcm or less), and to have a moderately high PTC effect (10<sup>3</sup> or higher) in order to withstand a direct current (DC) voltage of 16 to 20 volts. Polyolefins, particularly 20 polyethylene (PE)-based conductive materials, have been widely explored and employed in these low DC voltage applications.

Polymeric PTC sensor devices that are capable of operating at much higher voltages, such as the 110 to 130 25 alternating current voltages (VAC) ("Line" voltages) present in AC electrical lines, in which the effective AC current may 30 have peaks equivalent to 156 to 184 DC volts have recently been developed by Therm-O-Disc, Inc. Such polymeric PTC devices have been found to be particularly useful as self-resettable sensors to protect AC motors from damage caused by over-temperature or over-current surge. For example, and without limitation, such high voltage capacity polymeric PTC devices would be useful to protect the motors of household appliances, such as dishwashers, washers, refrigerators and the like.

In view of the foregoing, there is a need for the development 35 of polymeric PTC compositions and devices comprising them that exhibit a high PTC effect, have a low initial resistivity, that exhibit substantial electrical and thermal stability, and that are capable of use over a broad voltage range, i.e., from about 6 volts to about 300 volts.

### SUMMARY OF THE INVENTION

The invention provides polymeric PTC compositions and 45 electrical PTC devices having increased voltage capabilities while maintaining a low RT resistance. In particular, the polymeric compositions also demonstrate a high PTC effect (the resistivity at the  $T_s$  is at least 10<sup>4</sup> to 10<sup>5</sup> times the resistivity at 25° C.) and a low initial resistivity at 25° C. (preferably 10 Ωcm or less, more preferably 5 mΩ or less).

The electrical PTC devices comprising these polymeric PTC 50 compositions preferably have a resistance at 25° C. of 500 mΩ or less (preferably about 5 mΩ to about 500 mΩ, more preferably about 7.5 mΩ to about 200 mΩ, typically about 10 mΩ to about 100 mΩ) with a desirable design geometry, and can withstand a voltage of 110 to 130 VAC or greater without failure for at least 4 hours, preferably up to 24 hours or more, after reaching the  $T_s$ .

The polymeric PTC compositions of the invention, demonstrating the above characteristics, comprise an organic 60 polymer, a particulate conductive filler, an inert filler including fibrillated fibers and, optionally, an additive selected from the group consisting of inorganic stabilizers, flame retardants, antioxidants, antiozonants, accelerators, pigments, foaming agents, crosslinking agents and dispersing agents. The compositions may or may not be crosslinked 65 to improve electrical stability before or after their use in the electrical PTC devices of the invention. Preferably, the

polymer component of the composition has a melting point ( $T_m$ ) of 100° C. to 200° C. and the PTC composition exhibits a thermal expansion coefficient of  $4.0 \times 10^{-4}$  to  $2.0 \times 10^{-3}$  cm/cm° C. at a temperature in the range of  $T_m$  to  $T_m$  minus 10° C.

The electrical PTC devices of the invention have, for example, the high voltage capability to protect equipment operating on Line current voltages from over-heating and/or over-current surges. The devices are particularly useful as self-resetting sensors for AC motors, such as those of household appliances, such as dishwashers, washers, refrigerators and the like. Additionally, PTC compositions for use in low voltage devices such as batteries, actuators, disk drives, test equipment and automotive applications are also described below.

#### BRIEF DESCRIPTION OF THE DRAWINGS

FIG. 1 is a schematic illustration of a PTC chip comprising the polymeric PTC composition of the invention sandwiched between two metal electrodes.

FIG. 2 is a schematic illustration of an embodiment of a PTC device according to the invention, comprising the PTC chip of FIG. 1 with two attached terminals.

#### DETAILED DESCRIPTION OF THE INVENTION

The PTC polymeric composition of the present invention comprises an organic polymer, a particulate conductive filler, an inert filler including fibrillated fibers and, optionally, an additive selected from the group consisting of flame retardants, stabilizers, antioxidants, antiozonants, accelerators, pigments, foaming agents, crosslinking agents, coupling agents, co-agents and dispersing agents. While not specifically limited to high voltage applications, for purposes of conveying the concepts of the present invention, PTC devices employing the novel PTC polymeric compositions will generally be described with reference to high voltage embodiments. The criteria for a high voltage capacity polymeric composition are (i) a high PTC effect, (ii) a low initial resistivity at 25° C., and (iii) the capability of withstanding a voltage of 110 to 130 VAC or greater while maintaining electrical and thermal stability. As used herein, the term "high PTC effect" refers to a composition resistivity at the  $T_s$  that is at least  $10^4$  to  $10^5$  times the composition resistivity at room temperature (for convenience, 25° C.). There is no particular requirement as to the temperature at which the composition switches to its higher resistivity state. That is, the magnitude of the PTC effect has been found to be more important than the  $T_s$ .

As used here, the term "low initial resistivity" refers to an initial composition resistivity at 25° C. of 100  $\Omega$ cm or less, preferably 10  $\Omega$ cm or less, more preferably 5  $\Omega$ cm or less, especially 2  $\Omega$ cm or less, thus providing for a PTC device having a low resistance at 25° C. of about 500 m $\Omega$  or less, preferably about 5 m $\Omega$  to 500 m $\Omega$ , more preferably about 7.5 m $\Omega$  to about 10 m $\Omega$  to about 200 m $\Omega$ , typically about 10 m $\Omega$  to about 100 m $\Omega$ , with an appropriate geometric design and size, as discussed further below.

The organic polymer component of the composition of the present invention is generally selected from a crystalline organic polymer, an amorphous thermoplastic polymer (such as polycarbonate or polystyrene), an elastomer (such as polybutadiene or ethylene/propylene/diene (EPDM) polymer) or a blend comprising at least one of these. Suitable crystalline polymers include polymers of one or more olefins, particularly polyethylene; copolymers of at

least one olefin and at least one monomer copolymerisable therewith such as ethylene acrylic acid, ethylene ethyl acrylate and ethylene vinyl acetate; melt shapeable fluoropolymers such as polyvinylidene fluoride and ethylene tetrafluoroethylene and blends of two or more such crystalline polymers.

Other polymeric components of the composition of the present invention (i.e., nylon-12 and/or nylon-11) are disclosed in the co-pending U.S. patent applications Ser. Nos. 08/729,822 now U.S. Pat. No. 5,837,114 and 09/046,853 now U.S. Pat. No. 5,985,182, incorporated by reference above. Preferred organic polymer components include high density polyethylene and nylons, such as nylon-11, nylon-12 or polyvinylfluoride, by way of non-limiting example. Nylon-11 and/or nylon-12 based conductive compositions have very high switching temperatures ( $T_s$  greater than 125° C., preferably between 140° C. and 200° C., and typically between 150° C. and 195° C.). Moreover, many of these compositions demonstrate a high PTC effect of greater than  $10^4$ , an initial resistivity of 100  $\Omega$ cm or less at 25° C., especially 10  $\Omega$ cm or less, thus providing for a PTC device having a low resistance of about 500 m $\Omega$  or less, preferably about 5 m $\Omega$  to about 500 m $\Omega$ , more preferably about 7.5 m $\Omega$  to about 200 m $\Omega$ , typically about 10 m $\Omega$  to about 100 m $\Omega$ , with an appropriate geometric design and size.

It is known that the  $T_s$  of a conductive polymeric composition is generally slightly below the melting point ( $T_m$ ) of the polymeric matrix. If the thermal expansion coefficient of the polymer is sufficiently high near the  $T_m$ , a high PTC effect may occur. Further, it is known that the greater the crystallinity of the polymer, the smaller the temperature range over which the rapid rise in resistivity occurs. Thus, crystalline polymers exhibit more "squareness", or electrical stability, in a resistivity versus temperature curve.

The preferred crystalline or semi-crystalline polymer component in the conductive polymeric composition of the present invention has a crystallinity in the range of 20% to 70%, and preferably 25% to 60%. In order to achieve a composition with a high PTC effect, it is preferable that the polymer has a melting point ( $T_m$ ) in the temperature range of 100° C. to 200° C. and the PTC composition has a high thermal expansion coefficient value at a temperature in the range  $T_m$  to  $T_m$  minus 10° C. of about  $4.0 \times 10^{-4}$  to about  $2.0 \times 10^{-3}$  cm/cm° C. Preferably, the polymer substantially withstands decomposition at a processing temperature that is at least 20° C. and preferably less than 120° C. above the  $T_m$ .

The crystalline or semi-crystalline polymer component of the conductive polymeric composition of the invention may also comprise a polymer blend containing, in addition to the first polymer, between about 0.5 to 50.0% of a second crystalline or semi-crystalline polymer based on the total polymeric component. The second crystalline or semi-crystalline polymer is preferably a polyolefin-based or polyester-based thermoplastic elastomer. Preferably the second polymer has a melting point ( $T_m$ ) in the temperature range of 100° C. to 200° C. and a high thermal expansion coefficient value at a temperature in the range  $T_m$  to  $T_m$  minus 10° C. that is at least four times greater than the thermal expansion coefficient value at 25° C.

The particulate electrically conductive filler may comprise carbon black, graphite, metal particles, or a combination of these. Metal particles may include, but are not limited to, nickel particles, silver flakes, or particles of tungsten, molybdenum, gold, platinum, iron, aluminum, copper, tantalum, zinc, cobalt, chromium, lead, titanium, tin alloys or mixtures of the foregoing. Such metal fillers for use in conductive polymeric compositions are known in the art.

It is preferred to use medium to high structured carbon black with a relatively low resistivity. Examples of carbon black are Sterling N550, Vulcan XC-72, and Black Pearl 700, all available from Cabot Corporation, Norcross, Ga. A suitable carbon black, such as Sterling SO N550, has a particle size of about 0.05 to 0.08 microns, and a typical structure at 110-130 volts of  $10^{-5} \text{ m}^3/\text{kg}$  as determined by dibutylphthalate (DBP) absorption. The particulate conductive filler ranges from 15.0 phr to 150 phr and, preferably, from 60.0 phr to 120.0 phr.

The inert filler component comprises fibrillated fibers made from a variety of materials including, but not limited to, polypropylene, polyether ketone, acryl synthetic resins, polyethylene terephthalate, polybutylene terephthalate, cotton and cellulose. By "fibrillated fibers", it is meant that the fibers have a large number of small fibrils (branches) extending from the main fiber. Preferred commercially available fibrillated fibers are fibrillated Kevlar® fibers, sold under product designation no. 1F543 by DuPont.

Other inert fibers may be employed in association with the fibrillated fibers described above. Among the useful fibers are continuous and chopped fibers including, by way of non-limiting example, fiberglass and polyamide fibers such as Kevlar (available from DuPont). Such fibers may be randomly oriented or, preferably, will be specifically oriented to improve the anisotropic behavior. The total amount of fibers employed, including either fibrillated fibers alone or a combination of fibrillated and non-fibrillated fibers which generally range from between about 0.25 phr to about 50.0 phr and, preferably, from about 0.5 phr to about 10.0 phr. It should be understood that "phr" means parts per 100.0 parts of the organic polymer component.

Additional inert fillers may also be employed including, for example, amorphous polymeric powders such as silicon, nylons, fumed silica, calcium carbonate, magnesium carbonate, aluminum hydroxide, kaolin clay, barium sulphate, talc, chopped glass or continuous glass, among others. The inert filler component ranges from 2.0 phr to about 50.0 phr and, preferably, from 4.0 phr to about 12.0 phr.

In addition to the crystalline or semi-crystalline polymer component, the particulate conductive filler and the inert filler including fibrillated fibers, the conductive polymeric composition may additionally comprise additives to enhance electrical, mechanical, and thermal stability. Suitable inorganic additives for electrical and mechanical stability include metal oxides, such as magnesium oxide, zinc oxide, aluminum oxide, titanium oxide, or other materials, such as calcium carbonate, magnesium carbonate, alumina trihydrate, and magnesium hydroxide, or mixtures of any of the foregoing. Organic antioxidants may be optionally added to the composition to increase the thermal stability. In most cases, these are either phenol or aromatic amine type heat stabilizers, such as N,N'-1,6-hexanediylbis (3,5-bis (1,1-dimethylethyl)-4-hydroxy-benzene) propanamide (Irganox-1098, available from Ciba-Geigy Corp., Hawthorne, N.Y.), N-stearoyl-4-aminophenol, N-lauroyl-4-aminophenol, and polymerized 1,2-dihydro-2,2,4-trimethyl quinoline. The proportion by weight of the organic antioxidant agent in the composition may range from 0.1 phr to 15.0 phr and, preferably 0.5 phr to 7.5 phr. The conductive polymeric composition may also comprise other inert fillers, nucleating agents, antiozonants, fire retardants, stabilizers, dispersing agents, crosslinking agents, or other components.

To enhance electrical stability, the conductive polymer composition may be crosslinked by chemicals, such as

organic peroxide compounds, or by irradiation, such as by a high energy electron beam, ultraviolet radiation or by gamma radiation, as known in the art. Although crosslinking is dependent on the polymeric components and the application, normal crosslinking levels are equivalent to that achieved by an irradiation dose in the range of 1 to 150 Mrads, preferably 2.5 to 20 Mrads, e.g., 10.0 Mrads. If crosslinking is by irradiation, the composition may be crosslinked before or after attachment of the electrodes.

In an embodiment of the invention, the high temperature PTC device of the invention comprises a PTC "chip" 1 illustrated in FIG. 1 and electrical terminals 12 and 14, as described below and schematically illustrated in FIG. 2. As shown in FIG. 1, the PTC chip 1 comprises the conductive polymeric composition 2 of the invention sandwiched between metal electrodes 3. The electrodes 3 and the PTC composition 2 are preferably arranged so that the current flows through the PTC composition over an area L×W of the chip 1 that has a thickness, T, such that W/T is at least 2, preferably at least 5, especially at least 10. The electrical resistance of the chip or PTC device also depends on the thickness and the dimensions W and L, and T may be varied in order to achieve a preferable resistance, described below. For example, a typical PTC chip generally has a thickness of 0.05 to 5 millimeters (mm), preferably 0.1 to 2.0 mm, and more preferably, 0.2 to 1.0 mm. The general shape of the chip/device may be that of the illustrated embodiment or may be of any shape with dimensions that achieve the preferred resistance.

It is generally preferred to use two planar electrodes of the same area which are placed opposite to each other on either side of a flat PTC polymeric composition of constant thickness. The material for the electrodes is not specially limited, and can be selected from silver, copper, nickel, aluminum, gold and the like. The material can also be selected from combinations of these metals, nickel-plated copper, tin-plated copper, and the like. The electrodes are preferably used in a sheet form. The thickness of the sheet is generally less than 1 mm, preferably less than 0.5 mm, and more preferably less than 0.1 mm.

The high temperature PTC device manufactured by compression molding or by extrusion/lamination, as described below, and containing a crosslinked composition demonstrates electrical stability. As termed herein, a device demonstrating "electrical stability" has an initial resistance  $R_o$  at 25° C. and a resistance  $R_x$  at 25° C. after X cycles to the switching temperature and back to 25° C., wherein the value of the ratio  $(R_x - R_o)/R_o$ , which is the ratio of the increase in resistance after X temperature excursion, to the initial resistance at 25° C. Generally speaking, the lower the value, the more stable the composition.

The conductive polymeric compositions of the invention are prepared by methods known in the art. In general, the polymer or polymer blend, the conductive filler, the inert filler including fibrillated fibers and additives (if appropriate) are compounded at a temperature that is at least 20° C. higher, but no more than 120° C. higher, than the melting temperature of the polymer or polymer blend. The compounding temperature is determined by the flow property of the compounds. In general, the higher the filler content (e.g., carbon black), the higher is the temperature used for compounding. After compounding, the homogeneous composition may be obtained in any form, such as pellets. The composition is then subjected to a hot-press or extrusion/lamination process and transformed into a thin PTC sheet.

To manufacture PTC sheets by compression molding, homogeneous pellets of the PTC composition are placed in

a molder and covered with metal foil (electrodes) on top and bottom. The composition and metal foil sandwich is then laminated into a PTC sheet under pressure. The compression molding processing parameters are variable and depend upon the PTC composition. For example, the higher the filler (e.g., carbon black) content, the higher is the processing temperature and/or the higher is the pressure used and/or the longer is the processing time. By controlling the parameters of temperature, pressure and time, different sheet materials with various thicknesses may be obtained.

To manufacture PTC sheets by extrusion, process parameters such as the temperature profile, head pressure, RPM, and the extruder screw design are important in controlling the PTC properties of resulting PTC sheet. Generally, the higher the filler content, the higher is the processing temperature used to maintain the head pressure. A screw with a straight-through design is preferred in the manufacture of PTC sheets. Because this screw design provides low shear force and mechanical energy during the process, the possibility of breaking down the carbon black aggregates is reduced, resulting in PTC sheets having low resistivity. The thickness of the extruded sheets is generally controlled by the die gap and the gap between the laminator rollers. During the extrusion process, metallic electrodes in the form of metal foil covering both the top and bottom of a layer of the polymer compound, are laminated to the composition. Compositions, such as those described below in the Examples, that contain nylon-12 (or nylon-11), carbon black, magnesium oxide, and the like, in varying proportions, are processed by extrusion/lamination.

PTC sheets obtained, e.g., by compression molding or extrusion, are then cut to obtain PTC chips having predetermined dimensions and comprising the conductive polymeric composition sandwiched between the metal electrodes. The composition may be crosslinked, such as by irradiation, if desired, prior to cutting of the sheets into PTC chips. Electrical terminals are then soldered to each individual chip to form PTC electrical devices.

A suitable solder provides good bonding between the terminal and the chip at 25° C. and maintains a good bonding at the switching temperature of the device. The bonding is characterized by the shear strength. A shear strength of 250 Kg or more at 25° C. for a 2x1 cm<sup>2</sup> PTC device is generally acceptable. The solder is also required to show a good flow property at its melting temperature to homogeneously cover the area of the device dimension. The solder used generally has a melting temperature of 10° C., preferably 20° C. above the switching temperature of the device. Examples of solders suitable for use in the invention high temperature PTC devices are 63Sn/37Pb (Mp: 183° C.), 96.5Sn/3.5Ag (Mp: 221° C.) and 95Sn/5Sb (Mp: 240° C.), all available from Lucas-Milhaupt, Inc., Cudahy, Wis.; or 96Sn/4Ag (Mp: 230° C.) and 95Sn/5Ag (Mp: 245° C.), all available from EFD, Inc., East Providence, R.I.

The following examples illustrate embodiments of the high voltage capacity conductive polymeric PTC compositions and electrical PTC devices of the invention. However, these embodiments are not intended to be limiting, as other methods of preparing the compositions and devices e.g., injection molding, to achieve desired electrical and thermal properties may be utilized by those skilled in the art. The compositions, PTC chips and PTC devices were tested for PTC properties directly by a resistance versus temperature (R-T) test and indirectly by a switching test, overvoltage test, cycle test, and stall test, as described below. The number of samples tested from each batch of chips is indicated below and the results of the testing reported in

Table 1. The resistance of the PTC chips and devices is measured, using a four-wire standard method, with a micro-ohmmeter (e.g., Keithley 580, Keithley Instruments, Cleveland, Ohio) having an accuracy of  $\pm 0.01 \text{ M}\Omega$ .

The cycle test is performed in a manner similar to the switching test, except that the switching parameters (voltage and amperage) remain constant during a specified number of switching cycle excursions from -40° C. to the T<sub>s</sub> and back to -40° C. The resistance of the device is measured at 25° C. before and after a specified number of cycles. The initial resistance at 25° C. is designated R<sub>o</sub> and the resistance after X numbers of cycles is designated R<sub>x</sub>, e.g. R<sub>100</sub>. The resistance increase ratio is (R<sub>x</sub>-R<sub>o</sub>)/R<sub>o</sub>.

The cycling test is a way to evaluate the electrical stability of the polymeric PTC devices. The test is conducted at -40° C. for 1000 cycles. The devices are switched at 30 volts and 6.2 amps. The cycle consists at 2 minutes in the switched state with one minute intervals between cycles. The resistance of the device is measured before and after the cycling.

As reflected below, the overvoltage testing is conducted by a stepwise increase in the voltage starting at 5 volts. Knee voltage as the phrase is used below is a well known measure indicative of the voltage capability of the device.

## EXAMPLES

### Example 1

Using the formulas shown in Table 1, the compounds were mixed for 15 minutes at 180° C. in a ml brabender internal mixer. The compounds were then placed between nickel coated copper foil and compression molded at 10 tons for 15 minutes at 190° C. The sheet of PTC material was then cut into 11 by 20 mm chips and dip soldered to attach leads.

TABLE 1

| Compounds in (phr) parts per 100.0 parts of the polymeric component |           |           |           |
|---------------------------------------------------------------------|-----------|-----------|-----------|
|                                                                     | Control A | Control B | Example 1 |
| HDPE                                                                | 100       | 100       | 100       |
| Carbon Black N550                                                   | 75        | 75        | 75        |
| MgO                                                                 | 6         | 6         | 6         |
| Agerite MA                                                          | 3         | 3         | 3         |
| Standard Fiber (6F561)                                              | 0         | 3         | 0         |
| Fibrillated Fiber (1F543)                                           | 0         | 0         | 3         |
| <u>Overvoltage Testing*</u>                                         |           |           |           |
| Device Resistance (mOhms RT)                                        | 24.4      | 25.9      | 26.1      |
| Knee Voltage (DC)                                                   | 48.6      | 62.0      | 70.8      |
| <u>Cold Cycling (1000 cycles @-40OC)**</u>                          |           |           |           |
| Device Resistance (mOhms RT)                                        | 27.3      | 25.5      | 29.2      |
| Resistance Increase (%)                                             | 607       | 522       | 526       |

\*Avg. of five samples

\*\*Avg. of two samples

As can be seen from a review of Table 1, by employing the fibrillated fibers, the voltage capability of the sample device is significantly increased without significantly increasing the resistance of the device. Generally, an increase in voltage capability also involves increasing the resistance of a device either by increasing the thickness of the device or decreasing the carbon black content.

The use of fibrillated fibers improves the trade off between device resistance and voltage capability. As seen in Example 1 use of the fibrillated fibers (Example 1) exhibited a knee voltage increase of 22.2% while maintaining the initial

device resistance as compared to Control A which did not contain any fibers. Use of the fibrillated fibers also exhibited a significant advantage over standard randomly oriented fibers (Control B) with a knee voltage increase of 14%.

Another apparent advantage of using the fibrillated fibers is their ability to improve the voltage stability of the polymeric PTC device. After cold cycling, the PTC devices containing the fibrillated fibers had a significantly lower resistance increase than control compound A.

While the invention has been described herein with reference to the preferred embodiments, it is to be understood that it is not intended to limit the invention to the specific forms disclosed. On the contrary, it is intended to cover all modifications and alternative forms falling within the spirit and scope of the invention.

We claim:

1. A polymeric PTC composition comprising an organic polymer, a conductive filler; an inert filler including fibrillated fibers and, optionally, one or more additives selected from the group consisting of flame retardants, stabilizers, antioxidants, antiozonants, accelerators, pigments, foaming agents, crosslinking agents, coupling agents, co-agents and dispersing agents.

2. The composition of claim 1, wherein the polymer includes a crystalline or semi-crystalline polymer.

3. The composition of claim 1 wherein the organic polymer includes at least one polymer selected from the group consisting of high density polyethylene, nylon-11, nylon-12, polyvinylidene fluoride and mixtures or copolymers thereof.

4. The composition of claim 1, wherein the polymer has a melting point,  $T_m$  of 100° C. to 250° C.

5. The composition of claim 4, wherein the composition exhibits a thermal expansion co-efficient of  $4.0 \times 10^{-4}$  to  $2.0 \times 10^{-3}$  cm/cm\*°C at a temperature in the range of  $T_m$  to  $T_m$  minus 10° C.

6. The composition of claim 1, having a resistivity at 25° C. of 100 Ωcm or less.

7. The composition of claim 1, wherein said inert filler is present in an amount of between about 0.25 phr to 50.0 phr.

8. The composition of claim 1, wherein said inert filler is present in an amount of between about 0.5 phr to 10.0 phr.

9. The composition of claim 1, wherein the conductive filler is selected from the group consisting of carbon black, graphite, metal particles, and mixtures thereof.

10. The composition of claim 9, wherein the metal particles are selected from the group consisting of nickel particles, silver flakes, or particles of tungsten, molybdenum, gold, platinum, iron, aluminum, copper, tantalum, zinc, cobalt, chromium, lead, titanium, tin alloys, and mixtures thereof.

11. The composition of claim 1, wherein the inorganic stabilizers are selected from the group consisting of magnesium oxide, zinc oxide, aluminum oxide, titanium oxide, calcium carbonate, magnesium carbonate, alumina trihydrate, magnesium hydroxide, and mixtures thereof.

12. The composition of claim 1, wherein the antioxidant comprises a phenol or an aromatic amine.

13. The composition of claim 12, wherein the antioxidant is selected from the group consisting of N,N'-1,6-hexanediylbis (3,5-bis (1,1-dimethylethyl)-4-hydroxybenzene) propanamide, (N-stearoyl-4-aminophenol, N-lauroyl-4-aminophenol, polymerized 1,2-dihydro-2,2,4-trimethyl quinoline, and mixtures thereof.

14. The composition of claim 1 wherein said particulate conductive filler is present in an amount of between about 15.0 phr to 150.0 phr.

15. The composition of claim 1 wherein said particulate conductive filler is present in an amount of between about 60.0 phr to 120.0 phr.

16. The composition of claim 1, wherein the polymeric composition is crosslinked with the aid of a chemical agent or by irradiation.

17. The composition of claim 1, further comprising between about 0.5% to 50.0% of a second crystalline or semi-crystalline polymer based on the total polymeric component.

18. The composition of claim 17 wherein the second polymer has a melting temperature  $T_m$  of about 100° C. to about 250° C.

19. The composition of claim 17, wherein the second polymer has a thermal expansion co-efficient value at a temperature in the range of  $T_m$  to  $T_m$  minus 10° C. that is at least four times greater than the thermal expansion co-efficient value at 25° C.

20. The composition of claim 17, wherein the second polymer is selected from a polyolefin-based or a polyester-based thermoplastic elastomer, and mixtures and copolymers thereof.

21. The composition of claim 1 wherein said polymeric PTC composition has a resistivity at its switching temperature that is at least  $10^4$  to  $10^5$  times the resistivity at 25° C., the composition being able to withstand a voltage of 110 to 130 VAC or greater while maintaining electrical and thermal stability.

22. An electrical device which exhibits PTC behavior, comprising:

(a) a conductive polymeric composition that comprises a crystalline or semi-crystalline polymer, a conductive filler, an inert filler including fibrillated fibers and, optionally, one or more additives selected from the group consisting of flame retardants, stabilizers, antioxidants, antiozonants, accelerators, pigments, foaming agents, crosslinking agents and dispersing agents, the composition having a resistivity at 25° C. of 100 Ωcm or less and a resistivity at its switching temperature that is at least  $10^4$  to  $10^5$  times the resistivity at 25° C.; and

(b) at least two electrodes which are in electrical contact with the conductive polymeric composition to allow a DC or an AC current to pass through the composition under an applied voltage, wherein the device has a resistance at 25° C. of 500 mΩ or less with a desirable design geometry.

23. The device of claim 22 wherein said device can withstand a voltage of 110 to 130 VAC or greater without failure for at least 4 hours after reaching its switching temperature.

24. The device of claim 22 wherein the device has a resistance at 25° C. of about 5.0 mΩ to about 400 mΩ.

25. The device of claim 22 wherein the device has a resistance at 25° C. of about 10 mΩ to about 100 mΩ.

26. The device of claim 22 wherein the organic polymer includes at least one polymer selected from the group consisting of high density polyethylene nylon-11, nylon-12, polyvinylidene fluoride and mixtures or copolymers thereof.

27. The device of claim 22, further comprising an electrical terminal soldered to an electrode by a solder having a melting temperature at least 10° C. above the switching temperature of the composition.

28. The device of claim 22, wherein the solder has a melting point of about 180° C. or greater.

29. The device of claim 22, wherein the solder has a melting point of about 220° C. or greater.

30. The device of claim 22 wherein the said inert filler is present in an amount of between about 0.25 phr to 50.0 phr.

**11**

**31.** The device of claim **22** wherein the said inert filler is present in an amount of between about 0.5 phr to 10.0 phr.

**32.** The device of claim **22** further comprising between about 0.5% to 50.0% of a second crystalline or semi-crystalline polymer based on the total polymeric component.

**33.** The device of claim **32** wherein the second polymer is selected from a polyolefin based or a polyester-based thermoplastic elastomer.

**34.** The device of claim **22** produced by compression molding.

**35.** The device of claim **22** produced by extrusion/lamination.

**12**

**36.** The device of claim **22** produced by injection molding.

**37.** The device of claim **22**, having an initial resistance  $R_o$  at 25° C. and a resistance  $R_y$  at 25° C. after Y minutes of stall at 110 to 130 VAC and the value of  $(R_y - R_o)/R_o$  is less than 1.5 times the  $R_o$ .

**38.** The device of claim **22**, having an initial resistance  $R_o$  at 25° C. and a resistance  $R_x$  at 25° C. after X cycles to the switching temperature and back to 25° C., and the value of  $(R_x - R_o)/R_o$  is less than three times the  $R_o$ .

\* \* \* \* \*

UNITED STATES PATENT AND TRADEMARK OFFICE  
**CERTIFICATE OF CORRECTION**

PATENT NO. : 6,197,220 B1  
DATED : March 6, 2001  
INVENTOR(S) : Edward J. Blok et al.

Page 1 of 1

It is certified that error appears in the above-identified patent and that said Letters Patent is hereby corrected as shown below:

Title page.

Under Attorney, Agent or Firm, "Harnes" should be -- Harness --.

Column 1.

Line 8, after "In" please insert -- particular, --.

Column 4.

Line 60, "conducive" should be -- conductive --.

Column 5.

Line 55, "1,1-" should be -- I,I --.

Column 9.

Line 33, "cm/cm\*C" should be -- cm/cm°C --.

Signed and Sealed this

Sixteenth Day of April, 2002

Attest:

Attesting Officer



JAMES E. ROGAN  
Director of the United States Patent and Trademark Office